



US007427344B2

(12) **United States Patent**  
**Han et al.**

(10) **Patent No.:** **US 7,427,344 B2**  
(45) **Date of Patent:** **\*Sep. 23, 2008**

(54) **METHODS FOR DETERMINING ORGANIC COMPONENT CONCENTRATIONS IN AN ELECTROLYTIC SOLUTION**

(75) Inventors: **Jianwen Han**, Danbury, CT (US); **MacKenzie E. King**, Southbury, CT (US)

(73) Assignee: **Advanced Technology Materials, Inc.**, Danbury, CT (US)

(\*) Notice: Subject to any disclaimer, the term of this patent is extended or adjusted under 35 U.S.C. 154(b) by 322 days.

This patent is subject to a terminal disclaimer.

(21) Appl. No.: **11/318,129**

(22) Filed: **Dec. 23, 2005**

(65) **Prior Publication Data**

US 2006/0102475 A1 May 18, 2006

**Related U.S. Application Data**

(62) Division of application No. 10/833,194, filed on Apr. 27, 2004, now Pat. No. 6,984,299.

(51) **Int. Cl.**  
**C25D 21/14** (2006.01)

(52) **U.S. Cl.** ..... **205/81**; 205/83; 205/101;  
205/296; 205/787

(58) **Field of Classification Search** ..... 205/81,  
205/83, 101, 296, 787  
See application file for complete search history.

(56) **References Cited**

U.S. PATENT DOCUMENTS

2,707,166 A 4/1955 Brown et al.  
2,707,167 A 4/1955 Hoover et al.  
2,830,014 A 4/1958 Gundel et al.  
2,884,366 A 4/1959 Anderson et al.

2,898,282 A 8/1959 Flook, Jr. et al.  
3,101,305 A 8/1963 Roth et al.  
3,276,979 A 10/1966 Strauss et al.  
3,288,690 A 11/1966 Creutz et al.  
3,655,534 A 4/1972 Kampe  
3,725,220 A 4/1973 Kessler

(Continued)

FOREIGN PATENT DOCUMENTS

DE 19911447 A1 12/2000

(Continued)

OTHER PUBLICATIONS

Bard, Allen J., et al., *Electrochemical Methods: Fundamentals and Applications*, 2nd Edition, 2001, pp. 15-16, Publisher: John Wiley & Sons, Inc., Published in : New York.

(Continued)

*Primary Examiner*—Susy Tsang-Foster

*Assistant Examiner*—William T Leader

(74) *Attorney, Agent, or Firm*—Steven J. Hultquist; Intellectual Property/Technology Law; Maggie Chappuis

(57) **ABSTRACT**

The present invention relates to a method and apparatus for determining organic additive concentrations in a sample electrolytic solution, preferably a copper electroplating solution, by measuring the double layer capacitance of a measuring electrode in such sample solution. Specifically, the present invention utilizes the correlation between double layer capacitance and the organic additive concentration for concentration mapping, based on the double layer capacitance measured for the sample electrolytic solution.

**20 Claims, 1 Drawing Sheet**



## U.S. PATENT DOCUMENTS

|                |         |                          |                 |         |               |
|----------------|---------|--------------------------|-----------------|---------|---------------|
| 3,798,138 A    | 3/1974  | Ostrow et al.            | 6,984,299 B2    | 1/2006  | Han et al.    |
| 3,883,414 A    | 5/1975  | Fujinaga et al.          | 7,022,215 B2    | 4/2006  | Schomburg     |
| 3,910,830 A    | 10/1975 | Mayse                    | 7,094,323 B2    | 8/2006  | King et al.   |
| 3,950,234 A    | 4/1976  | Faulkner et al.          | 2002/0070708 A1 | 6/2002  | Wu            |
| 3,972,789 A    | 8/1976  | Eppensteiner et al.      | 2003/0080000 A1 | 5/2003  | Robertson     |
| 3,996,124 A    | 12/1976 | Eaton et al.             | 2004/0040842 A1 | 3/2004  | King et al.   |
| 4,038,161 A    | 7/1977  | Eckles et al.            | 2004/0055888 A1 | 3/2004  | Wikiel et al. |
| 4,071,429 A    | 1/1978  | Wagenknecht et al.       | 2004/0065561 A1 | 4/2004  | Chalyt et al. |
| 4,119,532 A    | 10/1978 | Park                     | 2005/0016847 A1 | 1/2005  | Buehler       |
| 4,132,605 A    | 1/1979  | Tench et al.             | 2005/0067304 A1 | 3/2005  | King et al.   |
| 4,260,950 A    | 4/1981  | Hadden et al.            | 2005/0109624 A1 | 5/2005  | King et al.   |
| 4,305,039 A    | 12/1981 | Steuernagel et al.       | 2005/0224370 A1 | 10/2005 | Liu et al.    |
| 4,317,002 A    | 2/1982  | Spicer                   | 2005/0241948 A1 | 11/2005 | Han et al.    |
| 4,388,165 A    | 6/1983  | Koshiishi et al.         | 2005/0247576 A1 | 11/2005 | Tom et al.    |
| 4,496,454 A    | 1/1985  | Berger                   | 2006/0266648 A1 | 11/2006 | King et al.   |
| 4,498,039 A    | 2/1985  | Galwey et al.            |                 |         |               |
| 4,529,495 A    | 7/1985  | Marsoner                 |                 |         |               |
| 4,568,445 A    | 2/1986  | Cates et al.             |                 |         |               |
| 4,589,958 A    | 5/1986  | Alexander et al.         |                 |         |               |
| 4,595,462 A    | 6/1986  | Vangaever et al.         |                 |         |               |
| 4,707,378 A    | 11/1987 | McBride et al.           |                 |         |               |
| 4,772,375 A    | 9/1988  | Wullschleger et al.      |                 |         |               |
| 4,812,210 A    | 3/1989  | Bonivert et al.          |                 |         |               |
| 4,849,330 A    | 7/1989  | Humphries et al.         |                 |         |               |
| 4,917,774 A    | 4/1990  | Fisher                   |                 |         |               |
| 4,917,777 A    | 4/1990  | Fisher                   |                 |         |               |
| 5,017,860 A    | 5/1991  | Germer et al.            |                 |         |               |
| 5,074,157 A    | 12/1991 | Marsoner et al.          |                 |         |               |
| 5,131,999 A    | 7/1992  | Gunasingham              |                 |         |               |
| 5,162,077 A    | 11/1992 | Bryan et al.             |                 |         |               |
| 5,192,403 A    | 3/1993  | Chang et al.             |                 |         |               |
| 5,223,118 A    | 6/1993  | Sonnenberg et al.        |                 |         |               |
| 5,268,087 A    | 12/1993 | Lu                       |                 |         |               |
| 5,288,387 A    | 2/1994  | Ito et al.               |                 |         |               |
| 5,296,123 A    | 3/1994  | Reddy et al.             |                 |         |               |
| 5,316,649 A    | 5/1994  | Kronberg                 |                 |         |               |
| 5,320,721 A    | 6/1994  | Ludwig et al.            |                 |         |               |
| 5,325,038 A    | 6/1994  | Banzai et al.            |                 |         |               |
| 5,352,350 A    | 10/1994 | Andricacos et al.        |                 |         |               |
| 5,404,018 A    | 4/1995  | Yasuda et al.            |                 |         |               |
| 5,447,802 A    | 9/1995  | Tobiyama et al.          |                 |         |               |
| 5,462,645 A    | 10/1995 | Albery et al.            |                 |         |               |
| 5,612,698 A    | 3/1997  | Reay                     |                 |         |               |
| 5,635,043 A    | 6/1997  | Turyan et al.            |                 |         |               |
| 6,022,470 A    | 2/2000  | Yarnitzky                |                 |         |               |
| 6,210,640 B1   | 4/2001  | Ruth et al.              |                 |         |               |
| 6,231,743 B1   | 5/2001  | Etherington              |                 |         |               |
| 6,254,760 B1   | 7/2001  | Shen et al.              |                 |         |               |
| 6,270,651 B1   | 8/2001  | Essalik et al.           |                 |         |               |
| 6,280,602 B1   | 8/2001  | Robertson                |                 |         |               |
| 6,288,783 B1   | 9/2001  | Auad                     |                 |         |               |
| 6,365,033 B1   | 4/2002  | Graham et al.            |                 |         |               |
| 6,366,794 B1   | 4/2002  | Moussy et al.            |                 |         |               |
| 6,395,152 B1   | 5/2002  | Wang                     |                 |         |               |
| 6,409,903 B1   | 6/2002  | Chung et al.             |                 |         |               |
| 6,458,262 B1   | 10/2002 | Reid                     |                 |         |               |
| 6,459,011 B1   | 10/2002 | Tarr et al.              |                 |         |               |
| 6,478,950 B1   | 11/2002 | Peat et al.              |                 |         |               |
| 6,495,011 B2   | 12/2002 | Robertson                |                 |         |               |
| 6,558,519 B1   | 5/2003  | Dodgson et al.           |                 |         |               |
| 6,569,307 B2   | 5/2003  | Blachier et al.          |                 |         |               |
| 6,572,753 B2   | 6/2003  | Chalyt et al.            |                 |         |               |
| 6,592,737 B1   | 7/2003  | Robertson                |                 |         |               |
| 6,645,364 B2   | 11/2003 | Calvert et al.           |                 |         |               |
| 6,673,226 B1 * | 1/2004  | Kogan et al. .... 205/81 |                 |         |               |
| 6,709,568 B2   | 3/2004  | Han et al.               |                 |         |               |
| 6,758,955 B2   | 7/2004  | Robertson                |                 |         |               |
| 6,758,960 B1   | 7/2004  | Robertson                |                 |         |               |
| 6,808,611 B2   | 10/2004 | Sun et al.               |                 |         |               |
| 6,827,839 B2   | 12/2004 | Sonnenberg et al.        |                 |         |               |
| 6,974,531 B2   | 12/2005 | Andricacos et al.        |                 |         |               |

## FOREIGN PATENT DOCUMENTS

|    |                  |        |
|----|------------------|--------|
| EP | 0 302 009 A1     | 7/1988 |
| JP | 2001-073183 A    | 3/2001 |
| WO | WO - 01/29548 A1 | 4/2001 |

## OTHER PUBLICATIONS

Liu, Yonghui, Testing Technology of Electrochemistry, (English relevance attached), 1987, p. 159, Published in: Beijing.

Milchev, Alexander, et al., A glavanostatic study of electrochemical nucleation, Journal of Electroanalytical Chemistry, Aug. 1992, pp. 93-102, vol. 333, No. 1 and 2.

Oldham, Keith B., et al., Fundamentals of Electrochemical Science, 1994, pp. 328-332, Publisher: Academic Press, Inc., Published in: San Diego.

Alwash, S. H. et al., A rotating disc electrode with heat transfer facilities for corrosion studies, Corrosion Science, 1987, pp. 383-390, vol. 27, No. 4.

Barz, H., et al., Measurement of the surface temperature of rotating electrodes, J. Electroanal. Chem., 1976, pp. 415-418, vol. 69.

Cerna, N., Determination of chlorides in an acid copper-plating bath, Povrchove Upravy, 1973, pp. 11-12, vol. 13, No. 6.

Cheng, X. L., et al., Analysis of organic additives in copper-plating brightener by high performance liquid chromatography, Se. Pu., Nov. 1999, pp. 602-603, vol. 17, No. 6.

Dikusar, A. I., et al., Thermokinetic instability of electrode processes, J. Electroanal. Chem., 1986, pp. 11-23, vol. 207.

Freeman, J.E., et al., A fiber-optic absorption cell for remote determination of copper in industrial electroplating baths, Analytica Chimica Acta, 1985, pp. 121-128, vol. 177.

Freitag, Walter O., et al., Determination of the individual additive components in acid copper plating baths, Plat. Surf. Fin., Oct. 1983, pp. 55-60, vol. 70, No. 10.

Healy, John P., et al., The chemistry of the additives in an acid copper electroplating bath: Part II. The instability 4,5-dithiaoctane-1, ..., J. Electroanal. Chem., Oct. 1992, pp. 167-177, vol. 338, No. 1-2.

Healy, John P., et al., The chemistry of the additives in an acid copper electroplating bath: Part III. The mechanism of brightening by 4,5- ..., J. Electroanal. Chem., Oct. 1992, pp. 179-187, vol. 338, No. 1-2.

Hui Liang, Huang, et al., Flow potentiometric and constant-current stripping analysis for mercury(II) with gold, platinum and carbon fibre ..., Analytica Chimica Acta, 1987, pp. 1-9, vol. 201.

Kim, Jae Jeong, et al., Catalytic behavior of 3-mercaptopropane sulfonic acid on Cu electrodeposition and its effect on Cu film properties ..., J. Electronanal. Chem., Jan. 30, 2003, pp. 61-66, vol. 542, No. 1.

Kruglikov, S. S., et al., The effect of some primary and secondary brighteners on the double layer capacitance in nickel electrodeposition, Electrochimica Acta, Sep. 1967, pp. 1263-1271, vol. 12, No. 9.

Merriam-Webster's Collegiate Dictionary: 10th Ed., 1998, pp. 328, 361, 478.

METROHM, Product description of 731 Relay Box, Downloaded May 11, 2005 from <http://www.metrohm.com/products/05/acc/731/731.html>, May 11, 2005.

METROHM, Product description of 772 Pump Unit, Downloaded May 11, 2005 from <http://www.metrohm.com/products/05/acc/772/772.html>, May 11, 2005.

METROHM, Product description of MVA-3 voltammetry system, Downloaded May 11, 2005 from <http://www.metrohm.com/products/06/mva/mva03/mva03.html>, May 6, 2004.

METROHM, Product description of Titrando Dosino, <http://www.metrohm.com/titrando/products/units/800/800.html>, 2003.

METROHM, Product descripton of Titrando PC Control, Downloaded May 11, 2005 from <http://www.metrohm.com/titrando/products/control/pc/pc.html>, 2004.

Seisler, H.W., et al., Near Infrared Spectroscopy, Near Infrared Spectroscopy, 2002, Publisher: Wiley.

Skoog, Douglas A., et al., Principles of Instrumental Analysis, 3rd Ed., 1985, pp. 332-337, Publisher: Harcourt College Publishers.

Tench, Dennis, et al., Cyclic pulse voltammetric stripping analysis of acid copper plating baths, *J. Electrochem. Soc.*, Apr. 1985, pp. 831-834, vol. 132, No. 4.

Vereecken, P.M., et al., The chemistry of additives in damascene copper plating, *IBM J. Res. Dev.*, Jan. 2005, pp. 3-18, vol. 49, No. 1.

Wojciechowski, Marek, et al., Square-wave anodic stripping voltammetry of lead and cadmium at cylindrical graphite fiber microelectrodes with . . ., *Analytica Chimica Acta*, 1991, pp. 433-445, vol. 249, No. 2.

Wikipedia, Universal Serial Bus—Wikipedia , Downloaded May 11, 2005 from <http://en.wikipedia.org/wiki/USB>, May 11, 2005.

Wyche, et al., Constant low-voltage drop rotating electrode assembly, *Electrochemical Technology*, 1966, pp. 447, vol. 4, No. 7-8.

“Aldrich Handbook of Fine Chemicals and Laboratory Equipment”, 2003-2004, pp. 500, 501 and 1634, Publisher: Aldrich Chemical Co., Published in: Milwaukee, WI.

\* cited by examiner

**Figure 1**

## METHODS FOR DETERMINING ORGANIC COMPONENT CONCENTRATIONS IN AN ELECTROLYTIC SOLUTION

### CROSS-REFERENCE TO RELATED APPLICATIONS

This application is a divisional application of U.S. patent application Ser. No. 10/833,194, entitled "Methods For Determining Organic Component Concentrations In An Electrolytic Solution", filed on Apr. 27, 2004, and issued as U.S. Pat. No. 6,984,299 on Jan. 10, 2006.

### BACKGROUND OF THE INVENTION

#### 1. Field of the Invention

The present invention relates to methods and apparatuses for determining organic component concentrations in an electrolytic solution, and more specifically to determination of organic component concentrations in a copper electroplating solution.

#### 2. Description of the Related Art

In electrochemical deposition (ECD) process, the rigorous control of the relative proportions of respective inorganic and organic ingredients in the ECD bath is critical to the achievement of satisfactory results in the rate of metal film formation and the quality of the film so formed. During the use of the plating bath solution, the plating process may be affected by depletion of inorganic components and organic additives as well as by organic byproduct formation. The ECD bath chemistry therefore must be maintained by periodic replacement of a part or the entire ECD bath. It is therefore important to continuously or periodically monitor the concentrations of inorganic and/or organic components in the ECD bath, and responsively add respective components to the bath to maintain the composition of the bath in an effective state for the electrochemical deposition operation.

It is therefore one object of the present invention to provide an improved method for measuring concentrations of one or more organic components in an ECD bath.

Other objects and advantages will be more fully apparent from the ensuing disclosure and appended claims.

### SUMMARY OF THE INVENTION

The present invention in one aspect relates to a method for determining concentration of an organic component in a sample electrolytic solution. Such method comprises the steps of:

- applying a potential step to the sample electrolytic solution by using at least a working electrode and a reference electrode;
- measuring double layer capacitance of the working electrode in the sample electrolytic solution under the applied potential step; and
- determining the concentration of the organic component in the sample electrolytic solution, based on the double layer capacitance measured in step (b).

Another aspect of the present invention relates to an apparatus for measuring concentration of an organic component in a sample electrolytic solution, comprising:

- a measuring chamber containing a working electrode and a reference electrode, for receiving at least a portion of the sample electrolytic solution;
- an electrical source for applying a potential step to the sample electrolytic solution through the working and reference electrodes;

(c) means for measuring double layer capacitance of the working electrode in said sample electrolytic solution under the applied potential step; and

(d) computational means for determining the concentration of the organic component in said sample electrolytic solution, based on the double layer capacitance measured for the working electrode in the sample electrolytic solution.

Other aspects, features and embodiments of the present invention will be more fully apparent from the ensuing disclosure and appended claims.

### BRIEF DESCRIPTION OF THE DRAWINGS

FIG. 1 shows the current response curves measured for four different electrolytic solutions over time under an initial potential step of about -0.208V.

### DETAILED DESCRIPTION OF THE INVENTION, AND PREFERRED EMBODIMENTS THEREOF

The boundary between a measuring electrode and an electrolytic solution is called an interface. The electrolytic solution is a first phase in which charge is carried by the movement of ions, and the measuring electrode is a second phase in which charge is carried by the movements of electrons.

Two types of processes occur at the electrode-solution interface: (1) the faradaic process involves actual electron transfers between the measuring electrode and the electrolytic solution; and (2) the non-faradaic process involves adsorption and desorption of organic species onto and from the electrode surface where no charge actually cross the interface.

During non-faradaic process, although no charge actually cross the interface, external transient currents are present when the electrical potential, electrode surface area, or the composition of the electrolytic solution changes. These transient currents flow to charge or discharge the electrode-solution interfacial region, which is generally referred to as an electrical double layer.

The capacitance of such electrical double layer ( $C_d$ ) is a function of the applied electrical potential (E), the composition and concentration of the electrolytic solution, and the active electrode surface area. When the applied electrical potential and the active electrode surface area are constant, the double layer capacitance is directly correlative to the composition and concentration of the electrolytic solution.

Therefore, the present invention in one aspect provides a method for measuring the organic additive (i.e., suppressors, accelerators, and levelers) concentrations in a metal electroplating solution, more preferably a copper electroplating solution, based on the double layer capacitance of a working electrode that is immersed in such metal electroplating solution.

Under a given initial electrical potential or potential step (E), the metal electroplating solution demonstrates a current response that is characterized by an initial current peak or maximum current ( $I_{max}$ ) at initial time  $t_0$  and an exponentially decaying current (I) at subsequent time t, which are determined by:

$$I_{max} = \frac{E}{R_s}; \quad (1)$$

-continued

$$I = I_{max} \times e^{(-\frac{t}{R_s C_d})} \quad (II)$$

where  $R_s$  is the electrical resistance of the electrolytic solution, and  $e$  is the base for natural exponential.

When  $t=R_s C_d$ , the current  $I$  has decreased to about 37% of the initial current peak, as follows:

$$I = I_{max} \times e^{(-1)} = 0.368 \times I_{max} \quad (III)$$

The value of  $R_s C_d$  is usually referred to as the time constant  $t_c$ , which is characteristic to the given electrode-solution interface.

From equations (I)-(III), one can express the double layer capacitance  $C_d$  as:

$$C_d = \frac{t_c \times I_{max}}{E} \quad (IV)$$

Therefore, by measuring the current peak  $I_{max}$ , the time constant  $t_c$  required for the current to decrease to about 37% of the current peak  $I_{max}$ , and the initial potential step  $E$ , the double layer capacitance  $C_d$  of the measuring electrode in the sample electroplating solution can be determined quantitatively.

The current response of an electrolytic solution can be monitored by using one or more measuring devices. For example, an ammeter can be used to directly measuring the current flow through the sample electrolytic solution over time; alternatively, a combination of one or more potentiometers and one or more ohmmeters can be used to measuring the real-time potential and electrical resistance of the sample electrolytic solution, from which the current flow can be calculated.

Preferably, one or more calibration solutions are provided for constructing a correlative data set, which empirically correlates the double layer capacitance with the concentration of an organic component of interest. Specifically, each calibration solution so provided is compositionally identical to the sample electroplating solution but for the concentration of the organic component of interest, and each calibration solution preferably contains said organic component of interest at a unique, known concentration. The double layer capacitance of each calibration solution is measured according to the method described hereinabove and used in conjunction with the respective known concentration of the organic component of interest in each calibration solution to form the correlative data set.

Such correlative data set can then be used for direct mapping of the concentration of the organic component of interest in the sample electroplating solution, based on the double layer capacitance measured for such sample electroplating solution.

Preferably, the present invention employs a computer-based quantitative analyzer, which may comprise a computer,

central processor unit (CPU), microprocessor, integrated circuitry, operated and arranged to collect the current response data for determining the double layer capacitance of the sample solution and according to the method described hereinabove and for mapping the organic component concentration. More preferably, such quantitative analyzer has a correlative data set stored in its memory for direct concentration mapping based on the double layer capacitance measured for the sample solution. Alternatively, such quantitative analyzer comprises a capacitance-concentration correlation protocol for in situ construction of such a correlative data set based on current response data collected for various calibration solutions and the respective known organic component concentrations in such calibration solutions. The capacitance-concentration correlation protocol can be embodied in any suitable form, such as software operable in a general-purpose programmable digital computer. Alternatively, the protocol may be hard-wired in circuitry of a microelectronic computational module, embodied as firmware, or available on-line as an operational applet at an Internet site for concentration analysis.

Usage of double layer capacitance for determining organic component concentrations in the present invention is particularly advantageous for analysis of copper electroplating solutions. First, measurement of the double layer capacitance involves little or no reduction of the copper ions ( $Cu^{2+}$ ), because such measurement is carried out in a potential range that is lower than that required for  $Cu^{2+}$  reduction reaction, which protects the measuring electrode from being alloyed with the reduced copper and increases the useful life of the electrode. Further, since measurement of the double layer capacitance does not involve copper deposition, the organic additives contained in the sample electrolytic solution are not consumed, and the concentration of such organic additives in the electrolyte solution throughout the measurement cycles remains constant, therefore significantly increasing the reproducibility of the measurement results.

FIG. 1 shows the current response curves of four different electrolytic solutions, which include (1) a first electrolytic solution that contains copper sulfate, sulfuric acid, and chloride and is additive-free, (2) a second electrolytic solution that is compositionally identical to the first electrolytic solution but for containing a suppressor at a concentration of about 2.0 mL/L; (3) a third electrolytic solution that is compositionally identical to the first electrolytic solution but for containing an accelerator at a concentration of about 6.0 mL/L; (4) a fourth electrolytic solution that is compositionally identical to the first electrolytic solution but for containing a leveler at a concentration of about 2.5 mL/L.

An initial potential step ( $E$ ) of about -0.208V is applied to each of the above-listed electrolytic solutions, and the current response curves of the electrolytic solutions under such initial potential step are obtained.

The current peak ( $I_{max}$ ) and the time constant ( $t_c$ ) required for the current ( $I$ ) to drop from the peak value to about 37% of the peak value can be directly read from such current response curves, and from which the double layer capacitance ( $C_d$ ) can be calculated, according to equation (IV) provided hereinabove.

Following is a table listing the measurements obtained from the current response curves shown in FIG. 1.

|                                            |      | Solution (1) | Solution (2) | Solution (3) | Solution (4) |
|--------------------------------------------|------|--------------|--------------|--------------|--------------|
| Potential Step (E)                         |      | -0.208 V     | -0.208 V     | -0.208 V     | -0.208 V     |
| Current Peak (I <sub>max</sub> )           | Ave. | -77.6 nA     | -45.1 nA     | -58.1 nA     | -73.8 nA     |
|                                            | RSD  | -0.20%       | -1.50%       | -0.50%       | -0.50%       |
| Time Constant (t <sub>c</sub> )            |      | 0.065 sec.   | 0.0749 sec.  | 0.0586 sec.  | 0.0684 sec.  |
| Double Layer Capacitance (C <sub>d</sub> ) |      | 24.2 nF      | 16.2 nF      | 16.4 nF      | 24.3 nF      |
| Capacitance Change Rate                    |      | 0%           | -33%         | -32%         | 0.04%        |

Among the three organic additives tested, the suppressor as added into solution (2) has the greatest impact on the double layer capacitance, and the leveler as added into solution (4) has the least impact at the given concentration. Therefore, different organic additives have relatively different impact on the double layer capacitance, which can be used for distinguishing said organic components from one another.

While the invention has been described herein with reference to specific aspects, features and embodiments, it will be recognized that the invention is not thus limited, but rather extends to and encompasses other variations, modifications and alternative embodiments. Accordingly, the invention is intended to be broadly interpreted and construed to encompass all such other variations, modifications, and alternative embodiments, as being within the scope and spirit of the invention as hereinafter claimed.

What is claimed is:

1. A method for determining concentration of an organic component in a sample electrolytic solution, said method comprising the steps of:

- (a) applying a potential step to the sample electrolytic solution by using at least a working electrode and a reference electrode;
- (b) measuring double layer capacitance of the working electrode in said sample electrolytic solution under the applied potential step;
- (c) determining the concentration of the organic component in said sample electrolytic solution, based on the double layer capacitance measured in step (b), and
- (d) adding organic component when the concentration of organic component falls below effective electrolytic solution levels,

wherein the sample electrolytic solution comprises a copper electroplating solution comprising copper ions, and wherein the copper ions do not deposit onto the working electrode;

wherein the double layer capacitance of the working electrode is measured by monitoring current response of the sample electrolytic solution under the potential step over time; and

wherein the current response is measured using at least one measuring device selected from the group consisting of potentiometers, ammeters and ohmmeters.

2. The method of claim 1, wherein the organic component comprises an organic additive selected from the group consisting of suppressors, accelerators, and levelers.

3. The method of claim 1, wherein one or more calibration solutions containing said organic component at unique, known concentrations are provided, wherein the double layer capacitance of the working electrode in each of said calibration solutions under the potential step is measured, which is correlated to the concentration of the organic component in respective calibration solution, and wherein the concentration of the organic component in the sample electrolytic solution is determined based on the double layer capacitance mea-

sured for said sample electrolytic solution and the capacitance-concentration correlation obtained by measuring the calibration solutions.

4. The method of claim 3, wherein said one or more calibration solutions are compositionally identical to said sample electrolytic solution but for the organic component concentration.

5. The method of claim 1, wherein the double layer capacitance (C<sub>d</sub>) of the working electrode is determined by:

$$C_d = \frac{I_c \times I_{max}}{E}$$

wherein E is the applied potential step, I<sub>max</sub> is the current peak observed under said applied potential step E, and t<sub>c</sub> is a time constant, which is equal to the time required for the current to drop from I<sub>max</sub> to about 0.368×I<sub>max</sub>.

6. A method for determining concentration of an organic component in a sample electrolytic solution, said method comprising the steps of:

- (a) applying a potential step to the sample electrolytic solution by using at least a working electrode and a reference electrode;
- (b) measuring double layer capacitance of the working electrode in said sample electrolytic solution under the applied potential step;
- (c) determining the concentration of the organic component in said sample electrolytic solution, based on the double layer capacitance measured in step (b), and
- (d) adding organic component when the concentration of organic component falls below effective electrolytic solution levels,

wherein the sample electrolytic solution comprises a copper electroplating solution comprising copper ions, and wherein the copper ions do not deposit onto the working electrode;

wherein one or more calibration solutions containing said organic component at unique, known concentrations are provided, wherein the double layer capacitance of the working electrode in each of said calibration solutions under the potential step is measured, which is correlated to the concentration of the organic component in respective calibration solution, and wherein the concentration of the organic component in the sample electrolytic solution is determined based on the double layer capacitance measured for said sample electrolytic solution and the capacitance-concentration correlation obtained by measuring the calibration solutions; and

wherein the capacitance-concentration correlation data set is stored in a memory of a computational assembly.

7. The method of claim 6, wherein said computation assembly comprises an assembly selected from the group consisting of computers, central processing units (CPUs), microprocessors, and integrated circuitry.

8. The method of claim 6, wherein said computational assembly maps concentration of the organic component in said sample electrolytic solution based on the measured double layer capacitance and a correlative data set that empirically correlates double layer capacitance with concentration of the organic component.

9. The method of claim 6, wherein the capacitance-concentration correlation data set is constructed in situ by said computational assembly according to a capacitance-concentration correlation protocol.

10. The method of claim 6, wherein the organic component comprises an organic additive selected from the group consisting of suppressors, accelerators, and levelers.

11. The method of claim 6, wherein said one or more calibration solutions are compositionally identical to said sample electrolytic solution but for the organic component concentration.

12. The method of claim 6, wherein the double layer capacitance of the working electrode is measured by monitoring current response of the sample electrolytic solution under the potential step over time.

13. The method of claim 6, wherein the double layer capacitance ( $C_d$ ) of the working electrode is determined by:

$$C_d = \frac{t_c \times I_{max}}{E}$$

wherein E is the applied potential step,  $I_{max}$  is the current peak observed under said applied potential step E, and  $t_c$  is a time constant, which is equal to the time required for the current to drop from  $I_{max}$  to about  $0.368 \times I_{max}$ .

14. A method for determining concentration of an organic component in a sample electrolytic solution, said method comprising the steps of:

- (a) applying a potential step to the sample electrolytic solution by using at least a working electrode and a reference electrode;
- (b) measuring double layer capacitance of the working electrode in said sample electrolytic solution under the applied potential step;
- (c) determining the concentration of the organic component in said sample electrolytic solution, based on the double layer capacitance measured in step (b), and
- (d) adding organic component when the concentration of organic component falls below effective electrolytic solution levels,

wherein the sample electrolytic solution comprises a copper electroplating solution comprising copper ions, and wherein the copper ions do not deposit onto the working electrode; and

5 15 wherein the organic additives contained in the sample electrolytic solution are not consumed during the measurement of the double layer capacitance.

16. The method of claim 14, wherein organic component comprises an organic additive selected from the group consisting of suppressors, accelerators, and levelers.

17. The method of claim 14, wherein one or more calibration solutions containing said organic component at unique, known concentrations are provided, wherein the double layer capacitance of the working electrode in each of said calibration solutions under the potential step is measured, which is correlated to the concentration of the organic component in respective calibration solution, and wherein the concentration of the organic component in the sample electrolytic solution is determined based on the double layer capacitance measured for said sample electrolytic solution and the capacitance-concentration correlation obtained by measuring the calibration solutions.

18. The method of claim 16, wherein said one or more calibration solutions are compositionally identical to said sample electrolytic solution but for the organic component concentration.

19. The method of claim 18, wherein the double layer capacitance of the working electrode is measured by monitoring current response of the sample electrolytic solution under the potential step over time.

20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 10000 10005 10010 10015 10020 10025 10030 10035 10040 10045 10050 10055 10060 10065 10070 10075 10080 10085 10090 10095 10100 10105 10110 10115 10120 10125 10130 10135 10140 10145 10150 10155 10160 101

UNITED STATES PATENT AND TRADEMARK OFFICE  
**CERTIFICATE OF CORRECTION**

PATENT NO. : 7,427,344 B2  
APPLICATION NO. : 11/318129  
DATED : September 23, 2008  
INVENTOR(S) : Jianwen Han

Page 1 of 1

It is certified that error appears in the above-identified patent and that said Letters Patent is hereby corrected as shown below:

Cover page, item [75], inventors, "MacKenzie E. King" should be -- Mackenzie E. King --.

Signed and Sealed this

Thirtieth Day of December, 2008



JON W. DUDAS  
*Director of the United States Patent and Trademark Office*